# EUROPEAN PATENT SPECIFICATION

(11) **EP 0 115 910 B1**
(45) Date of publication and mention of the grant of the patent: **08.04.1987**
(21) Application number: 84300116.5
(22) Date of filing: 09.01.1984
(51) Int. Cl.: H01B 3/00

(54) **High voltage electrical apparatus**
Elektrische Hochspannungsvorrichtung
Dispositif électrique à haute tension

(30) Priority: 10.01.1983 GB 8300535
(43) Date of publication of application: 15.08.1984
(73) Proprietor: BICC Public Limited Company, London, WC1B 3QN (GB)
(72) Inventor: Pinching, Albert Arthur, Wood Green London N22 4BY (GB)
(74) Representative: Poole, Michael John

## Description

This invention relates to electrical apparatus in which a heat shrunk body of insulating material is subjected to an electrical stress along its surface of at least 10⁴V/m.

The use of plastics materials for such bodies, especially out of doors, is severely inhibited by the liability of many such materials to failure by "tracking" (the formation of conductive paths by carbonisation of the organic constituent(s) of the plastics material), rapid erosion, or flame.

A number of rigid materials that avoid premature failure of this kind have been developed, but availability of flexible materials and more especially heat-shrinkable materials is very limited; the most popular flexible materials currently commercially available are expensive materials based on the use of alumina trihydrate filler either in very large amounts or in combination with iron (III) oxide (which presumably catalyses some reaction that competes with carbonisation). Large amounts of filler limit physical properties that can be achieved, whereas iron (III) oxide imparts an undesirable intrinsic colour.

It is, of course, well known to use calcium carbonate as filler in insulating materials for electric cables. It is almost universally adopted in low-voltage insulating compositions based on polyvinyl chloride, but also known in other polymers and at higher voltages (e.g. GB-A-1151405 in which the polymer base is ethylene-propylene rubber). In cable applications, however, the requirements for physical properties are less exacting than for heat-shrink components, and high electrical stresses along the surface of the insulating material (as distinct from normal to that surface) and very carefully avoided. Cable insulating compositions do not therefore require resistance to the breakdown mode known as "tracking" which is characteristic of a longitudinally electrically stressed solid/gas interface.

GB-A-1464367 proposes the use of calcium carbonate filler in 'insulators' based on unsaturated polyester resins (which would be extremely rigid), but positively teaches that the use of alumina trihydrate as well is necessary if arc resistance is required (p. 2 lines 48-50). Arc resistance is not the same as resistance to tracking, but is another requirement for high-voltage components that will have a high stress along the surface, and so this document is positively teaching that compositions in which calcium carbonate is the only filler are suitable only for low-voltage applications.

JP-A-43-6526 teaches that certain olefin polymer compositions containing calcium carbonate have anti-tracking characteristics, but only when compounded with a certain proportion of carbon black, which precludes the preparation of pale or brightly coloured products.

DE-A-3038526 describes compositions for heat-shrunk applications which also contain carbon black as well as calcium carbonate, and is fully consistent with the teaching of the Japanese document.

GB-A-1551540 teaches compositions for heat-shrinkable articles in which calcium carbonate may be the only filler, but there is no suggestion that the articles would be suitable for any high-voltage application, and all the examples relate to accessories for telecommunication cables in which there would be no appreciable electrical stress at all.

GB-A-2019412 teaches compositions based on particular grades of polyethylene, in some of which (including at least one said to be suitable for heat-shrinkable sleeving) calcium carbonate is the only major filler. It also teaches that the compositions can be modified to make them suitable or high voltage insulational but that the addition of an anti-tracking filler is necessary for this purpose. There is no suggestion that heat-shrink and anti-tracking properties can be achieved in the same composition.

We have now discovered that certain compositions (known per se in general terms) can be heat-shrinkable, after shrinking are highly resistant to tracking and because calcium carbonate is used as the only substantial filler, may be pale or by the use of suitably chosen pigments, brightly coloured.

In accordance with the present invention, electrical apparatus in which a heat-shrunk body of insulating material is subjected to an electrical stress along its surface of at least 10⁴ V/m is characterised by the fact that the said body comprises particulate calcium carbonate dispersed as the only substantial filler in a compatible thermoplastic or elastomeric carbon-chain polymer matrix in an amount sufficient to raise the failure voltage of the body (as determined by the tracking resistance test method set out in ASTM specification D-2303) to a value not less than 3.0 kV.

By the use of the present invention, ultimate breakdown voltages in the range 4-6.2 kV have been attained; it is entirely surprising that such excellent tracking resistance can be achieved by the use of an inexpensive, white and apparently inert filler.

Commercially available filler grades of calcium carbonate, which generally have a mean particle size in the range 0.01-50 micrometre (but preferably below 10 micrometre) can be used, and comparable results are obtained with natural and synthetic (precipitated) types. Relatively coarse crushed limestone is also effective in raising failure voltage, but may have a detrimental effect on physical properties.

The polymer matrix may be of any carbon-chain polymer (by which is meant a polymer not having any significant number of hetero-atoms in its main chain) or carbon-chain polymer mixture that is sufficiently inert and capable of accepting the loading of calcium carbonate required to achieve the specified tracking resistance. Preferred are hydrocarbon-chain polymers with side-chain hetero-atoms to enhance compatibility and loading capacity, and the most preferred side-chains are esters and other carboxylic groups. Typical preferred polymers are the semi-αrystaIIine copolymers of ethylene with vinyl acetate, ethyl acrylate, methyl acrylate, butyl acrylate and acrylic acid; amorphous copolymers of this class as well as ethylene-propylene copolymer rubbers and ethylene-propylene-diene terpolymer rubbers can also be used.

The minimum loading required and the maximum acceptable will vary to some extent with the type of - polymer matrix and with the size, shape and surface condition of the calcium carbonate particles. Usually however a loading of at least 40 parts by weight for each hundred parts by weight of polymer matrix (hereinafter abbreviated to phr) will be needed to achieve the defined tracking resistance and a loading over 120 phr is likely to result in poor mechanical properties. 50-90 phr is usually recommended and 80 phr may be considered a starting point for optimisation.

The calcium carbonate particles may be coated with a dispersing agent, such as calcium stearate or with a coupling agent, such as a silane or titanate, or an organic material polymerised in situ on the particles.

The polymeric matrix may have been crosslinked, preferably by irradiation, with or without the use of promoters (such as triallyl cyanurate, trimethylolpropane, trimethyacrylate, ethylene glycol diamethacrylate, or triallyl trimellitate); conventional crosslinking reagents, e.g. peroxides, can usually be used alternatively, with or without the same type of promoter.

Minor amounts of other conventional additives may be present, important examples being antioxidants, U.V. stabilisers, flame retardants and processing aids. Pigments can also be used but need to be chosen with care as some (notably titanium dioxide) have a deleterious effect on tracking properties.

Formulations in accordance with the invention may be used for the whole, or a superficial layer of, extruded and injection moulded heat-shrunk components for insulators, cable joints and terminations.

### Examples 1-11

The following table of examples illustrates the invention; in all cases the composition was moulded into electrically insulating bodies in the form of sheets, crosslinked by irradiation at 200 kGy (20 Mrad) and tested for tracking resistance according to ASTM D-2303:

The calcium carbonates used in the examples are as follows:-
Snowcal 7ML is a superfine whiting grade of natural calcium carbonate with a mean particle size of 2.9 micrometre and a particle distribution (by sieving) as follows:
   finer than 25 micrometres - practically 100%
   finer than 20 micrometres - 99%
   finer than 10 micrometres - 95%
   finer than 5 micrometres - 75%
   finer than 3 micrometres - 53%

Winnofil S is a precipitated calcium carbonate with a nominal particle size of 75 nm, surface coated with calcium stearate to inhibit agglomeration and promote dispersion.

The crushed limestone was specified only as passing 100% through No. 200 British Standard mesh.

In the Table, (t) denotes ultimate breakdown by tracking and (f) ultimate breakdown by flaming; in other cases the mode of ultimate breakdown has not yet been determined.

### Example 12

In a further example, a commercially available material (sold in the UK by BXL Plastics Limited under the designation BP D 2979 FR) analysing as 100 parts ethylene-ethyl acrylate polymer, 80 parts of a natural calcium carbonate (estimated range of particle sizes very approximately 0.5-2 micrometre), small amount of Flectol H, was moulded into similar sheet insulators. Comparable test results were as follows:
erosion inception voltage - 3.5 kV
ultimate breakdown voltage (by flaming) - 6.25 kV

## Claims

1. Electrical apparatus in which a heat-shrunk body of insulating material is subjected to an electrical stress along its surface of at least 10⁴ V/m distinguished by the fact that the said body comprises particulate calcium carbonate dispersed as the only substantial filler in a compatible thermoplastic or elastomeric carbon-chain polymer matrix in an amount sufficient to raise the failure voltage of the body as determined by the tracking resistance test method set out in ASTM specification D-2303 to a value not less than 3.0 kV.

2. Electrical apparatus as claimed in Claim 1 in which the matrix is of a hydrocarbon chain polymer with side-chain hetero-atoms.

3. Electrical apparatus as claimed in Claim 1 in which the polymer matrix is selected from the semicrystalline copolymers of ethylene with vinyl acetate, methyl acrylate, methyl acrylate, butyl acrylate and acrylic acid.

## Patentansprüche

1. Elektrische Vorrichtung bei der ein durch Hitze aufgeschrumpfter Körper aus isolierendem Material entlang seiner Oberfläche einer elektrischen Belastung von mindestens 10⁴ V/m ausgesetzt ist, dadurch gekennzeichnet, daß der Körper teilchenförmiges Kalzium-carbonat aufweist, das als einziger wesentlicher Füllstoff in einer verträglichen thermoplastischen oder elastomeren Kohlenstoffketen-Polymermatrix in einer Menge verteilt ist, die ausreicht, die Ausfallspannung des Körpers, die nach der in der ASTM-Vorschrift D-2303 dargelegten Methode zur Prüfung der Kriechstromfestigkeit festgestellt wird, auf einen Wert von mindestens 3,0 kV zu erhöhen.

2. Elektrische Vorrichtung nach Anspruch 1, dadurch gekennzeichnet, daß die Matrix aus Kohlenwasserstoffketten-Polymerisat mit Seitenketten-Heteroatomen besteht.

3. Elektrische Vorrichtung nach Anspruch 1, dadurch gekennzeichnet daß die polymere Matrix ein halbkristallines Copolymerisat aus Äthylen mit Vinylacetat, Äthylacrylat, Methylacrylat, Butylacrylat oder Acrylsäure enthält.

## Revendications

1. Appareil électrique, dans lequel le corps d'un matériau isolant, thermo-rétracté, est soumis à une contrainte électrique d'au moins 10⁴ Volts/mètre le long de sa surface, caractérisé par le fait que ledit corps comprend du carbonate de calcium en particules, dispersé en tant que seule matière de charge essentielle dans une matrice d'un polymère à chaîne carbonée, thermoplastique ou élastomère, compatible dans une proportion suffisante pour élever la tension de claquage du corps, telle que déterminée par la méthode du test de la résistance au cheminement, décrite dans la spécification ASTM D-2303, à une valeur au moins égale à 3 kilovolts.

2. Appareil électrique selon la revendiction 1, dans lequel la matrice est un polymère à chaîne hydrocarbonée, avec des hétéro-atomes disposés dans des chaînes latérales.

3. Appareil électrique selon la revendication 1, dans lequel la matrice de polymère est sélectrionnée parmi les copolymères semi-cristallins de l'éthelène avec l'acétate de vinyle, l'acrylate d'éthyle, l'acrylate de méthyle, l'acrylate de butyle et l'acide acrylique.
